

April 28, 1936.

J. TAYLOR

2,038,772

BLASTING CHARGE

Filed Feb. 19, 1934



INVENTOR.  
James Taylor

*Wager S. Brown*

ATTORNEY.

## UNITED STATES PATENT OFFICE

2,038,772

## BLASTING CHARGE

James Taylor, Saltcoats, Scotland, assignor to  
 Imperial Chemical Industries Limited, a corporation of Great Britain

Application February 19, 1934, Serial No. 712,050  
 In Great Britain December 15, 1933

5 Claims. (Cl. 102—7)

Explosives of the non-detonating type, such as blackpowder, cordite, and the like, undergo exothermic decomposition on the application of flame or on exposure to high temperature. This 5 decomposition, as is well known, results in the formation of products at high temperatures such as are capable of igniting methane-air and coal dust-air mixtures, and such explosives are not safe for use in fiery mines.

10 Accordingly devices have been proposed for blasting, wherein such explosives as would be too dangerous to use in the ordinary manner are confined in a pressure-resisting shell having a gas release means adapted to allow the gases to 15 escape when the internal pressure rises to a certain value. The amount of explosive placed within the shell is insufficient of itself to operate the device, but a gas-producing substance or mixture of substances is also included in the shell, 20 for example ammonium nitrate or a mixture of ammonium nitrate and ammonium chloride or oxalate.

The gas-producing mixtures hitherto proposed for the purpose described have disadvantages. 25 Thus with ammonium nitrate a temperature of at least 180° C. is required to cause its decomposition and the evolution of considerable quantities of gas, so that a comparatively large amount of heat is required and a correspondingly large 30 amount of explosive or heating composition such as blackpowder.

I have found that mixtures of sodium nitrite or potassium nitrite with ammonium chloride or ammonium sulphate, in a range of widely varying 35 proportions, provide self-sustaining gas producing mixtures which when confined in a rigid vessel of the type having a member adapted to permit emission of the gases at a predetermined and considerable pressure are capable of effecting blasting with safety in fiery or dusty mines.

The mixtures used according to my invention, when initiated under ordinary pressure, do not exhibit explosive properties, but sustain their own 40 decomposition. A small proportion of moisture 45 of the order of 0.5% is desirable for the reaction mixture to be easily initiated by the application of heat.

In putting my invention into effect, heat is supplied within the container to one portion of the mixture, for instance by means of a 30 grain powder fuse. Where loading is to take place in fiery or dusty mines, it is of course desirable to use a safety igniter of a kind incapable of igniting firedamp-air mixture.

50 It is far from necessary that the two materials

should be present in stoichiometrical proportions. The mixtures may be used in powder form or may be granular or compressed into cartridges and it is desirable that they be wrapped up in fireproofed paper. They may, if desired, be loaded into the 5 container in the mine itself.

It will be understood that the invention is not limited to the case of coal mining, but it is of particularly great value in that art since it not only provides a reliable method of blasting but 10 also facilitates the production of round coal.

The following is a description of a device embodying my invention, which is illustrated in the appended drawing.

15 Into one threaded end of a shouldered strong steel container (1) there is screwed a firing head (2) separated from the container (1) by a sealing washer (9) of fibre or other suitable material such that a seal which is gas tight even at high pressures is ensured. The firing head (2) is provided with electrodes (7) and (8) of which one (8) is in metallic connection with the firing head (2), while the other (7) is insulated from the firing head. The mounting of the insulated electrode (7) is such as to allow no gas leakage at 20 pressures up to about 25 tons per sq. in. Terminals (10) and (11) are provided for the electrodes, which are used in initiating the cartridge electrically. A protective steel cap (3) having an aperture (14) for the leads to the terminals from 25 the cable of the exploder or other suitable source of electrical energy is screwed on the firing head (2). The blasting charge (13) is introduced loosely into the tube in the requisite amount. On the shoulder of the container remote from the 30 firing head (2) there is placed a fibre or like sealing washer (6), the steel bursting disc (5) adapted to be ruptured at a predetermined pressure being held in position between the said washer and the hollow screwed-in cap (4), which 35 is pierced with suitable channels for the venting of the gases and the direction and distribution of the blast. An electric powder fuse or safety igniter (12) containing for example 30 grains blackpowder is used for ignition and provided 40 with long leads from the electrodes and positioned as shown in the drawing so that the flash is directed towards the firing head and initiation occurs near the end of the charge adjacent to 45 the cap (4). By so positioning the cap the tendency of the charge to be forced into a plug at the end nearest the cap (4) is overcome. In blasting, the assembly is placed in the borehole with the cap (4) as far in as possible, and the device 50

may if desired be tamped. It is then fired electrically.

For convenience the device has been shown in the upright position, but it will be understood that the charge (13) would only assume the position shown if the device were horizontal. In practice, the device can be used in any position, so long as there is effective contact between the fuse (12) and the charge (13).

The invention is illustrated by the following example.

*Example*

A rigid container of the kind used in blasting with carbon dioxide, of 370 cc. capacity and venting at a pressure of 12 tons/sq. in. is used. 220 gm. of an intimate mixture of sodium nitrite and ammonium chloride in the proportions of 69:53 is introduced.

A safety igniter is provided as a source of ignition within the container. In carrying out the blast the cartridge is loaded into the borehole with the venting device to the rear.

The charge fails to ignite a 9% methane-air mixture either e. g. when tested in the open wrapped in fireproof paper or when enclosed as for blasting.

The mixtures of my invention may thus safely be handled within the mine even when not loaded into the blasting device.

My invention is capable of many variations, which will be obvious to those skilled in the art, and all such variations are intended to be covered in the appended claims although not necessarily specifically described herein.

I claim:

1. A blasting device of the non-detonating, gas-generating kind in which a gas-producing agent is confined within a pressure-resisting shell having a member adapted to permit escape of the gases at a predetermined and considerable pressure, said gas-producing agent comprising a mixture of an alkali metal nitrite with an ammonium salt, said mixture being capable of producing ammonium nitrite.

2. A device as set forth in claim 1, in which the gas-producing agent comprises a mixture of an alkali metal nitrite with an ammonium salt selected from the group consisting of ammonium chloride and ammonium sulphate.

3. A device as set forth in claim 1, in which the gas-producing agent is in the form of particles of substantial size, e. g. is in granular form.

4. A device as set forth in claim 1, in which the gas-producing mixture is wrapped up in the form of a cartridge in fireproofed paper.

5. A device as set forth in claim 1, in which the gas-producing agent comprises sodium nitrite and ammonium chloride.

JAMES TAYLOR. 30